

## UNITED STATES PATENT OFFICE

WILLIAM H. FURNESS, OF NATIONAL PARK, NEW JERSEY, ASSIGNOR TO CELLOCILK COMPANY, OF PHILADELPHIA, PENNSYLVANIA, A CORPORATION OF DELAWARE

## ARTIFICIAL SILK AND THE MANUFACTURE THEREOF

No Drawing.

Application filed April 6, 1927. Serial No. 181,614.

This invention relates to artificial silk and the manufacture thereof, and its nature, objects and advantages will be best appreciated from the following.

5 Considered from the standpoint of the fabric to be manufactured therefrom, the thread of my invention is composed of non-adherent, flexible filaments having the transparency and luster and fineness of natural silk, giving the fabric made therefrom the "hand", "drape", "softness" and other properties which characterize a natural silk product.

From the standpoint of manufacture into fabric, the silk has the following advantages. It is characterized by low elongation over the entire range of load both wet and dry, and has substantially the same elongation (from 4 to 10%) in the wet as in the dry state (65% atmospheric humidity) and 10 at any intermediate degree of relative humidity normally obtaining. In this connection, the strength-elongation curve of the silk in the dry state, as shown on the standard Serigraph chart, is substantially parallel to 15 the base line for over half the breaking load, with no yield points, the rise in the curve as it approaches the breaking point being gentle and uniform. The elongation curve in the wet state is approximately parallel to that 20 of the dry, with no yield points. It is, therefore, possible commercially to weave, wind, knit, twist, size, or otherwise manipulate or treat the thread in the manufacturing operations without appreciable change in dimension or other physical properties. This makes 25 it possible to operate on a cotton yarn basis without producing defective cloth. It also eliminates much of the apparatus, certain 30 of the operations, and reduces the number 35 of operatives and care required at present in the manufacture of fabric from artificial silk. In addition to the economies in plant investment, labor, etc., thus effected, it is possible, if desired, to speed up the mill operations and 40 still further reduce costs.

It will be apparent that the properties of low elongation and sameness of elongation, both wet and dry, will ensure the production 45 of a fabric which will withstand all manipulations wet or dry, including washing, dye-

ing, finishing, etc., without elongation or permanent distortion. In addition, the silk cannot elongate during fabrication so as to become rigid or change its refractive index which would produce a "shiner" due to this 55 cause.

The silk, therefore, resembles natural silk, but can be worked like cotton yarn, and, among other things, differs from all yarns in that its elongation-humidity curve is 60 straight and parallel to the base for substantially all degrees of relative humidity. Its dry strength is approximately 70% higher than cotton yarn of equivalent size.

The foregoing and other advantages will 65 be readily appreciated by those skilled in the textile art, but, in addition, the high dry strength, flexibility, elasticity, and elongation characteristics of the silk constitute a combination of properties which makes it possible 70 to employ the fabric for new uses, such as for cord tires, air-craft fabrics, water-proofed fabrics, etc.

I believe the unique physical properties of 75 the thread are to be attributed to the fact that I employ cellulose solutions of such character that the original crystallite chains of the cellulose are dispersed in the liquid in approximately their original form, and that the cells of the gel precipitated therefrom during the formation of the filaments of the 80 thread are of such character and disposition that by stretching they may be collapsed and elongated with the crystallite chains substantially intact and largely extending longitudinally of the thread in overlapping relation and with the inter-cellular spaces largely 85 eliminated or reduced; the properties thus secured being retained throughout the remaining operations. 90

In consequence of the foregoing I obtain, on the one hand, the high tensile strength hereinbefore referred to, and, on the other hand, remove the extensibility due to the structure formed by the precipitation of the 95 gel in the formation of the filaments to the point where the thread has the elongation characteristics set forth.

In the making of the silk of my invention I prefer to proceed as follows: I prepare 100

a very concentrated solution of pure copper hydrate, ammonia and cellulose, preferably in about minimum dissolving proportions. By proceeding in this manner I keep down the quantity of ammonia required to a point where its detrimental effect on the cellulose is negligible. I then dilute the solution thus prepared with a substantially inert liquid such as water, employing an amount thereof such that the resultant solution may be directly spun into a precipitating bath, such as a caustic bath, with the production of filaments, which, in relation to the spinneret orifices, are very small, and which are practically immediately and completely solidified so that when they merge into the thread they do not adhere but remain readily separable. I have found that the best results are obtained when the initial solution is of approximately fifteen to twenty percent cellulose concentration, this being diluted with sufficient water so that the resultant solution contains four percent of cellulose. The caustic bath is preferably a twenty percent solution, although the degree of concentration is not critical and may be materially varied from that specified.

I believe that the precipitation from the said solution is of such nature that the gel, although formed immediately, is neither too hard or stiff, nor too soft, to be collapsed, elongated, and manipulated as herein described, and that the structure of the gel is probably in the form of large thin walled cells, the walls of which are constituted by the crystallite chains in substantially intact condition. Also, with this solution, I am enabled, if desired, to form by direct spinning (as distinguished from the well known "stretch spinning" method) filaments as fine as those of natural silk through relatively coarse spinneret holes. For example, I may directly spin filaments as fine as one and one-half denier and below from orifices as large as four and one-half to five thousandths of an inch. The thread may be spun without filament breakage very rapidly—as high as 80 or 90 yards per minute, which effects a great economy in cost of production—or very slowly—as low as 10 yards per minute—which secures advantages in doffing which will be pointed out.

I have mentioned that a four percent cellulose solution is preferred as giving the best results, particularly as to strength of the thread. Solutions lower in cellulose content work approximately as well, but approach instability, and solutions of greater content do not produce as strong a thread. I prefer not to exceed a five percent solution nor to use less than a three and one-half percent solution.

A further advantage is that age does not affect the solution, nor do the solutions have to be aged.

The thread which has been precipitated is then passed over a drawing wheel and around a second drawing wheel of larger diameter, the difference in diameter depending upon the size of spool employed, speed of operation, etc. From the second and larger wheel the thread is led to a cap twister and is wound and twisted on to a spool with the employment of a loop or balloon at the cap. The thread is put under tension and stretched during this operation by the larger or stretching wheel and by the centrifugal force of the loop. This stretching which is given to the thread is believed to elongate the cells and form them into the shape of overlapping fibers running lengthwise of the thread, with the intercellular space practically eliminated or at least greatly reduced. The tension should be sufficient to impart a stretch which will remove extensibility to the point hereinbefore mentioned. The stretch given is retained by the thread on the spool.

For reasons of mechanical expediency, I prefer to operate the spool spindle and also the cap at constant speed, and to the end that the thread shall not be injured, and that it may be laid on the spool of uniform denier throughout, I proceed as follows: I operate the cap at a speed slower than the speed of the spindle and at approximately the speed of the balloon of the yarn. In consequence of this when starting a spool, the only relative movement as between the cap and the thread is the inward movement of the thread. As the thread is laid up and the diameter of the spool increases, the cap lags slightly behind the balloon of the yarn, but the relative movement as between the cap and the yarn is now small and in a direction approximately parallel to the fibers of the yarn. In consequence of this, there is no liability of damage to the yarn, and, for all practical purposes, the tension is solely that due to the centrifugal force referred to, but because of variations due to increase in diameter of the spool which might otherwise result in some change in denier, I provide the second or stretching wheel hereinbefore mentioned, which, in conjunction with the balloon, removes the extensibility to the point where the resistance to further extension is great enough to enable me to lay up the thread on the spool with uniform size.

When the spool is filled, it may be "doffed" without interrupting the manufacture of the thread. This results from the fact that at all rates of drawing, the filaments are practically immediately and completely solidified, i. e., change from the liquid to the solid phase. Therefore, I am able to reduce the speed of the spindle, the cap, the drawing wheel, and the extrusion pump. By thus reducing the speed of production of the thread, I may break the thread after it passes over the second wheel and allow it to accumulate on a suitable plate without material loss while the

5 filled spool is being doffed and a new spool inserted, and may easily start the thread and restore normal drawing conditions. I prefer to simultaneously reduce the speed of the spindle, the cap, the drawing wheel, and the extrusion pump, in order to make even at the slow speeds necessary for doffing, a thread of substantially the same size as before, so that I may be able to start the thread on the new

10 10 spool, an appreciable difference in the size of the thread making it impossible to do so.

To facilitate further treatment of the thread I prefer that the spools shall have a removable head, and I take the filled spool, 15 remove the head, and unwind the thread from the spool in the direction of the unheaded end, subjecting the thread, as it is being unwound, to a washing medium applied so that the successive layers, as they are exposed by 20 unwinding, are subjected thereto. This I prefer to do by immersing the spool in a bath. The bath contains a small amount of caustic soda or other electrolyte which prevents the softening of the thread, or, stated in other 25 words, the bath is one in which the gel is stable. The bath removes the greater proportion of the caustic soda and other water soluble materials of the thread, the unwinding and resultant exposure of successive layers being 30 very effective for this purpose. As the thread is being unwound and leaves the bath, it is drawn through an acid bath which converts the copper hydroxide into a soluble copper salt and also liberates the combined water of 35 the cellulose hydrate, whereby the thread is greatly reduced in diameter (deflated). The deflated thread is wound upon a spool or cylinder, preferably revolving in an acid bath. It will, of course, be understood that as rapid- 40 ly as the thread is being unwound, it is drawn through the acid bath and wound upon the cylinder, all of these operations being carried on with the thread under sufficient tension to maintain the stretch which was previously 45 given in the forming operation.

The thread which is wound upon the said cylinder is washed and dried while on the cylinder, and, in order that the "cake" of thread may be uniformly washed, I prefer to so wind 50 it that the layers are of successively diminishing length, which will produce a cake, the edge or end portions of which taper with the same exposure and the same permeability of those portions as has the main body portion 55 of the cake. Thus, the cake is uniformly washed throughout its length. The washing is facilitated by perforating the cylinder.

As one means for producing a cake of the characteristics hereinbefore described, I may 60 employ a cylinder or a spool, the spindle portion of which is convexed or slanted at the edges.

Owing to the fact that the thread is completely deflated before winding on the cylinder, the change in physical dimension dur-

ing washing and drying is negligible, and the thread will not become tangled. Furthermore, I am thereby enabled to put on a cylinder a very large amount of thread—15,000 yards or upwards of 150 denier size—which effects further economy and simplicity. It will be seen that the conditions are such that the thread does not become injured nor the fibers broken.

The washed and dried thread is now ready 70 to soften, and, as one means for accomplishing this, I unwind it from the cylinder and wind it upon a twisting spool for the purpose of imparting a final twisting which, due to the change in position of the fibers produced, softens the thread. This is possible because 80 of the non-adherent character of the fibers. To accomplish this the cylinder on which the thread has been washed and dried is placed upon two rollers, one or both of which are 85 driven, the thread, as it leaves the cylinder, preferably passing over one of the rollers. By driving the cylinder in this fashion, I am enabled to lay up the thread on a twisting spool from the relatively heavy cylinder without 90 removing the remaining extensibility. An advantage incident to causing the thread to pass over one of the rollers is that this roller may be kept wet so as to size or otherwise treat the thread. By this procedure I 95 eliminate the skeining operations heretofore required for softening and treating the washed and dried thread, and I am enabled to market the product on the spool. This not only effects an economy in the manufacturing 100 operations, but also an economy for the mill ultimately using the thread, besides which the damage which frequently resulted to the thread in the handling and shipping of skeins is entirely obviated.

105 It might here be mentioned that the thread may be twisted and wound in the wet state without distortion or loss of flexibility.

Among other advantages the silk may be doubled with cotton yarn in such manner 110 that the strength of the yarn is approximately equal to the combined strength of the two threads which, due to the marked difference in the elongation between cotton yarn and the heretofore manufactured silk, has not been 115 possible.

The apparatus herein referred to is illustrated and claimed in my copending applications Serial Nos. 239,401, 239,402, 239,403, 239,404, 239,405 filed December 12, 1927.

120 The drawing mechanism, the driving mechanism, the differential cap speed device, and the apparatus for laying up cakes are not specifically claimed herein, as the same constitute subject matter respectively claimed in 125 the applications just above listed.

No claim is herein made to the specific method of operating the cap twister, as this forms subject matter of application No. 239,403.

No claim is herein made to the specific method of laying up cakes, as this forms subject matter of application No. 239,405.

No claim is herein made to the specific method of drawing and stretching the thread, as this forms subject matter of application No. 239,401.

I claim:—

1. As a new article of manufacture, artificial silk thread having approximately the same elongation wet as dry.

2. As a new article of manufacture, artificial silk thread having approximately the same elongation wet as dry and having no appreciable yield points in its elongation-strength curve, wet and dry.

3. As a new article of manufacture, artificial silk thread having approximately the same elongation for all degrees of relative humidity normally obtaining.

4. As a new article of manufacture, artificial silk thread having a low elongation over a wide range of load.

5. As a new article of manufacture, artificial silk thread having a low elongation over a wide range of load and approximately the same elongation wet as dry.

6. As a new article of manufacture, artificial silk thread having a high initial resistance to elongation.

7. As a new article of manufacture, artificial silk thread having no appreciable yield points in its elongation-strength curve, wet and dry.

8. As a new article of manufacture, a direct spun fine filament cupro-ammonium artificial silk thread of the order of the denier of natural silk.

9. As a new article of manufacture, a cupro-ammonium artificial silk thread spun from a cellulose solution containing an amount of inert liquid such that filaments of the order of natural silk may be directly spun.

10. As a new article of manufacture, an artificial silk thread spun from a cellulose solution containing an amount of inert liquid such that filaments of the order of natural silk may be directly spun from relatively large orifices.

11. As a new article of manufacture, an artificial silk thread spun from a cellulose solution containing an amount of inert liquid such as to produce a gel of coarse thin walled cell structure, the cells of which under tension may be elongated sufficiently to ensure a flexible thread characterized by marked resistance to further elongation.

12. As a new article of manufacture, an artificial silk thread spun from a cellulose solution containing an amount of inert liquid such as to produce a gel of coarse thin walled cell structure.

13. As a new article of manufacture, fine filament artificial silk thread spun from a cupro-ammonium solution of cellulose so di-

lute that the gel precipitated in filament form is immediately and completely solidified before the filaments merge whereby the filaments remain in individual, readily separable form.

14. As a new article of manufacture, artificial silk thread precipitated from a solution in which the crystallite chain structure of the original cellulose is retained.

15. As a new article of manufacture, artificial silk thread precipitated from a solution in which the crystallite chain structure of the original cellulose is retained with the cell structure elongated and collapsed.

16. As a new article of manufacture, artificial silk thread probably in which the crystallite chain structure of the original cellulose is retained and probably in which the cells have been elongated and collapsed with the crystallite chains largely extending lengthwise of the thread characterized by the following properties—flexibility; high tensile strength both wet and dry; resistance to elongation over a wide range of load; approximately the same elongation wet as dry and at all intermediate degrees of humidity; and the filaments of which do not adhere one to the other.

17. As a new article of manufacture, artificial silk thread spun from a solution made by diluting with water a solution of copper hydroxide, ammonia and cellulose in approximately minimum dissolving proportions.

18. As a new article of manufacture, artificial silk thread spun from a solution made by diluting with water a solution of copper hydroxide, ammonia and cellulose in approximately minimum dissolving proportions, the dilution being such that the final solution contains about 4% of cellulose.

19. As a new article of manufacture, artificial silk thread which in the process of manufacture is stretched to remove the extensibility whereby the product has approximately the same extensibility wet as dry.

20. As a new article of manufacture, artificial silk thread which in the process of manufacture has had removed therefrom its extensibility to the point where the product has approximately the same elongation wet as dry.

21. As a new article of manufacture, artificial silk thread which in the process of manufacture has had removed therefrom its extensibility to the point where the product is resistant to elongation over a wide range of load wet and dry.

22. As a new article of manufacture, artificial silk thread which in the process of manufacture has had removed therefrom its extensibility to the point where the product is resistant to elongation over a range of load such that it can be woven substantially on a cotton basis without producing defective cloth.

23. As a new article of manufacture, artificial silk thread which in the process of manufacture, has had removed therefrom the extensibility to the point where the product is 50 resistant to elongation over a range of load which permits of manufacturing operations such as winding, weaving, twisting, etc., without alteration in denier.
24. As a new article of manufacture, artificial silk thread treated in the manufacture 10 to remove extensibility to the point where the thread is so resistant to elongation even while wet that the thread may be sized in a manner customary to cotton yarn and fabricated without substantial distortion.
25. As a new article of manufacture, artificial silk thread which in the process of manufacture has had removed therefrom its extensibility to the point where the strength- 20 elongation relation curve of the product is substantially flat and parallel to the base line until the breaking point is approached and without yield points.
26. As a new article of manufacture, artificial silk thread which in the process of manufacture has had removed therefrom its extensibility to the point where the elongation-humidity curve of the product is straight and parallel the base for substantially all degrees 30 of humidity.
27. As a new article of manufacture, artificial silk thread which in the process of manufacture has had removed therefrom its extensibility to the point where the elongation- 35 strength curve in the wet state is without appreciable yield points.
28. As a new article of manufacture, artificial thread silk in which the extensibility due to the precipitation of a cellulose solution in 40 the form of a gel is largely removed in the process of manufacture thereof.
29. As a new article of manufacture, artificial thread silk in which the extensibility due to the precipitation of a cellulose solution in 45 the form of a gel is removed in the process of manufacture thereof to the point where the resultant thread is substantially incapable of a longitudinal distortion which would produce rigidity.
30. As a new article of manufacture, artificial silk thread in which the extensibility due to the precipitation of a cellulose solution in 50 the form of a gel is removed in the process of manufacture thereof to the point where the resultant thread is substantially incapable of a longitudinal distortion which would alter the refractive index of that thread in the finished cloth.
31. As a new article of manufacture, artificial silk thread in which the extensibility due 60 to the precipitation of a cellulose solution in the form of a gel is removed in the process of manufacture thereof to the point where the resultant thread is substantially incapable of a longitudinal distortion such as will
- substantially alter the denier size in the ordinary steps of winding, weaving, etc., on a cotton basis.
32. The process of making artificial silk, which includes spinning a cellulose solution 70 into a precipitating bath, and stretching the formed thread to the point where it has in the finished state approximately the same elongation wet as dry, a marked resistance to elongation over a wide range of load, approximately the same elongation for all degrees of relative humidity normally obtaining, and no appreciable yield points in its elongation curve.
33. The process of making cellulose thread 80 which consists in forming the thread, in deflating the thread, in winding the thread on a spool or cylinder, and then in washing and drying the thread while on the spool.
34. The method of spinning artificial silk 85 thread which comprises forming the thread, stretching the thread to largely remove extensibility, and removing water solubles and decopping and deflating and winding on a spool or cylinder, under sufficient tension to 90 retain the stretch given in removal of extensibility.
35. The process which comprises forming cellulose thread from individual and non-adherent filaments and in carrying out all subsequent operations such as washing and decopping while maintaining the filaments in 95 a non-adhesive condition.
36. The process which comprises forming cellulose thread, in winding and twisting it on a spool, in removing the spool, and in unwinding the thread therefrom while subjecting it to a washing medium and thereafter, as the unwinding proceeds, drawing the washed thread through a decopping solution, 100 and in winding the decopped thread as drawn on a spool or cylinder.
37. In the manufacture of cellulose thread, the step which comprises deflating the formed thread before winding on the washing spool 110 or cylinder to a point such that the thread suffers no material change in dimension in the final conditioning thereof, and in winding the deflated thread.
38. In the manufacture of cellulose thread, 115 the step which comprises deflating the formed thread to a point such that the thread suffers no material change in dimension in the final conditioning thereof, and in winding the thread into a cake and then in washing and 120 drying the cake.
39. The process of spinning, twisting and winding a large amount of artificial silk thread on a spool of relatively small diameter which comprises spinning the thread; removing extensibility of the thread to the point that the thread may be led on to the spool of uniform denier notwithstanding the 125 change in diameter of the spool, twisting the 130

thread and in winding the thread on the spool.

40. The process of spinning, twisting and winding a large amount of artificial silk thread on a spool of relatively small diameter which comprises spinning the thread; removing extensibility of the thread to the point that the thread may be led on to the spool of uniform denier notwithstanding the change in diameter of the spool, twisting the thread and in winding the thread on the spool under light tension.

In testimony whereof I have hereunto signed my name.

**WILLIAM H. FURNESS.**

**15**

**20**

**25**

**30**

**35**

**40**

**45**

**50**

**55**

**60**

**65**